

Patented Apr. 12, 1938

2,114,006

# UNITED STATES PATENT OFFICE

2,114,006

## ELECTRODEPOSITION OF METALS

Virgil H. Waite, Berea, Ohio, assignor to The McGean Chemical Company, Cleveland, Ohio, a corporation of Ohio

No Drawing. Original application August 15, 1934, Serial No. 740,021. Divided and this application August 5, 1936, Serial No. 94,437

18 Claims. (Cl. 204—14)

This invention relates to electrodeposition of metals; and it has to do more especially with electrodeposition of metals of the nickel group comprising nickel, cobalt and iron, employing plating baths or solutions containing an organic salt of the metal to be deposited, together with a relatively small quantity of an organic compound, particularly a sulfonic acid compound, as a catalyst, promoter, or assisting agent; the plating baths being operated relatively hot and at relatively low pH (hydrogen ion concentration); whereby electrodeposits of superior characteristics are produced. The invention comprises the novel process aforesaid, as well as the novel plating baths or solutions and the novel electrodeposits produced therefrom.

While the invention in its broader aspects is not restricted to electrodeposition of any particular metal or group of metals, but is applicable in a very wide field with varying degrees of utility, its greatest practical utility at the present time is in the electrodeposition of metals of the nickel group aforesaid, and preeminently of nickel itself. In explaining the underlying principles of the invention, therefore, reference will be made herein more particularly to nickel plating; but it will be understood that this is merely for purposes of illustration and that in its broader aspects the invention is of wider scope, as indicated.

A principal object of the invention is to produce electrodeposits of nickel or other metal which are bright and lustrous, i. e. image-reflecting or mirror-like. In the field of decorative plating, the final bright, glossy finish usually required and sought has usually been obtained heretofore by buffing nickeled articles, which are then given a thin coating of chromium, for example. This sequence of operations necessitates a re-racking of the articles between the nickel and chromium plating tanks, and, what is more important, also results in a loss of nickel removed by the buffing or mechanical polishing operation, not to mention the expense of the labor involved. A method of plating whereby the nickeled articles come from the bath with a bright and lustrous finish, such as is afforded by the present invention, is therefore highly desirable.

Another object of the invention is to attain the foregoing desirable results while at the same time permitting rapid deposition of relatively thick or heavy metal coatings as required by modern plating practice, and to do this relatively simply and economically.

With the foregoing objects in view, as well as others which will become apparent as the description proceeds, the invention consists in the novel plating processes and baths, as well as the resultant novel electrodeposits, which will

be described in certain concrete illustrative examples hereinafter and will then be more particularly pointed out in the appended claims.

It has been proposed heretofore to produce bright or image-reflecting deposits of nickel directly in the plating bath, but all such prior proposals have involved serious disadvantages rendering them unsuitable for economically successful application in actual practice. What little is to be found in the literature on the subject of bright nickel plating has to do with cold nickel solutions or baths operated at ordinary room temperature and producing relatively thin deposits. Although the use of certain addition agents, chiefly colloidal, as brighteners in nickel plating baths has been suggested heretofore, they have not been widely used because of the difficulty in controlling their effect and because of the very narrow range of operating conditions within which satisfactory deposits could be obtained even experimentally. Nickel and other metal solutions are very susceptible to the action of colloids, and the amounts used, as well as other details of operation, must be carefully regulated to avoid production of cracked and curled deposits. Due either to their inherent character or to the particular manner in which it has been recommended to use them, the addition agents heretofore suggested for use were operative only for low current densities and thin deposits and are therefore not available for use in the more recent plating practice which calls for the rapid deposition of relatively heavy coatings. Addition agents thus suggested heretofore have included a wide variety of organic compounds, as well as certain metals such as zinc or cadmium. But it has not been possible heretofore, by the use of any of those addition agents, as proposed, to obtain satisfactory bright deposits of appreciable thickness such, for example, as a thickness of more than 0.0002 inch; and even in the case of thinner deposits, an approach to satisfactory brightness or luster was obtainable only by operating at low current densities impractical or very undesirable to use in modern plating practice.

According to the present invention, nickel plating baths, for example, are employed which in most respects may much resemble those now commonly used but which contain one or more addition agents which serve to promote production of bright or mirror-like deposits, which novel baths are, furthermore, operated within a temperature range above ordinary room temperature and within a pH range that is relatively low (i. e. relatively strongly acid). The particular temperature and pH vary within the indicated ranges depending upon the particular addition agent or agents employed in any given plating bath, but may be adjusted and controlled in accordance

with the present invention to give optimum results. In general the process of the invention involves operating at bath temperatures ranging from about 35° C. to about 60° C., a range of 40° to 50° C. being found especially desirable in the case of most of the addition agents most suitable for practicing the invention. The pH of the plating baths may range from 5.5 to 1.5, a pH of approximately 2.5 being found especially suitable in the majority of cases. Under these conditions of plating bath control or adjustment, and with the use of a proper addition agent or agents, employment of relatively high current densities in producing thoroughly satisfactory coatings becomes feasible and is also characteristic of the invention in its best embodiments. Current densities of from 30 to 50 amperes per square foot are especially suitable and are typical, although in many cases current densities as high as 60 to 100 amperes per square foot are practical and desirable. Lower current densities, e. g. on the order of 10 amperes per square foot, are also permissible; and it is to be understood that the use of such lower current densities is within the scope of the invention in its broader aspects, although higher current densities can advantageously be employed, as above pointed out, and are preferred in practice.

In general, addition agents suitable for use in practicing the present invention comprise water-soluble organic compounds herein designated as sulfonated amino toluene compounds, including not only amino toluene (toluidine) sulfonic acids, but also suitable salts thereof and diamido di-35 methyl diphenyl (toluidine) sulfonic acids, as well as suitable salts thereof; compounds of this class having the amino group in the ortho position being especially suitable. It is also found that the desirable action of these agents is appreciably enhanced if they are mildly chlorinated, as, for example, by the use of a chlorine-in-water solution as the chlorinating agent. It is further found that in some cases especially good results are obtained when a small quantity of a metal promoter, e. g. zinc or cadmium, is associated in the bath with the addition agent. The organic agents may be used singly or in combinations of two or more within the scope of the invention; but from the standpoint of simplifying control of the composition of the plating solution, it is generally more desirable to employ only one. For the same reason, it is generally better to employ only one metal addition agent or promoter (in the form of a salt) in conjunction with one organic addition agent.

Another important feature of the invention in its best embodiments is the fact that the addition agent used is employed in only relatively very small quantity, so small indeed as not to combine with or bind chemically any substantial proportion of the amount of the plating metal present in the bath or solution to be deposited therefrom. In other words, in the practice of this invention, the metal to be deposited ordinarily exists in the bath wholly or almost wholly as a salt of an inorganic acid; but the term "inorganic acid" as here used is not intended to exclude the presence in the bath of variable proportions of acetate, formate, and/or oxalate, for example, of the plating metal, which salts may be employed as buffering agents. In other words, the organic addition agents as employed in the present invention seem to function very much in the role of catalysts in promoting the production of the 75 perior electrodeposits obtainable in the practice

of the invention, said addition agents being present in relatively small and generally only minute proportion, as compared with the amount of plating metal salt or salts in the bath and apparently undergoing very little depletion in operation except for the unavoidable drag-out. In referring to the action of these addition agents as catalytic, however, it is not intended thereby in any sense to rest the present invention upon a theoretical basis, but only to characterize conveniently and in a general way their promoting and assisting action, in contrast to the prior proposed use, in connection with tin, copper or lead plating, of certain sulfonic acid compounds in relatively large quantities for the purpose of binding chemically approximately half or more of the total plating metal present as a metal sulfonate. In contradistinction to methods heretofore proposed in applying the process of the invention to bright nickel plating, for example, the deposit may be made, and most desirably is made, at the relatively high temperatures and high current densities commonly employed commercially in ordinary non-bright nickel plating practice; and the luster of the deposit becomes greater with increase of the thickness of the deposit. In fact, the present process enables plating upon a surface which is originally dull and, by continuing the deposition for a sufficient length of time and thus obtaining a relatively thick deposit, securing a deposit that is image-reflecting or mirror-like. This remarkable result can be accomplished, moreover, by using nickel plating baths which, except for the employment of an addition agent or "catalyst" as herein described, have compositions otherwise usual in present commercial practice. A typical plating bath of this character may contain, for example, 180 to 360 grams of hydrated nickel sulfate, 8 to 75 grams of nickel chloride and 8 to 45 grams of boric acid, per liter of solution.

Among the specific organic addition agents which have been found especially desirable to employ as assistants or catalysts in accordance with the invention may be mentioned the following: 2 amino toluene 5 sulfonic acid and 2 amino toluene 4 sulfonic acid (o-toluidine sulfonic acids); 4 amino toluene 2 sulfonic acid (a p-toluidine sulfonic acid); and o-toluidine disulfonic acid. The products resulting from mild chlorination of these compounds are also very effective.

A bath containing any of the materials mentioned in the next preceding paragraph produces brighter deposits if the pH is decreased (acidity increased) down to pH of 2.5 or even lower in some instances; while increase of temperature up to approximately 45° C., or in some cases higher, also causes an increase in the brightness of the deposit. Moreover, the deposits so obtained are characterized by good adherence and substantial freedom from cracking or curling, these eminently satisfactory results being obtainable over a relatively wide working range of temperature, pH value and current density, within the limits hereinabove indicated.

It is of course to be understood that, in general, salts (e. g. the sodium or other alkali metal salts, the calcium salts, etc.) of the sulfonic acids mentioned not detrimental to the plating bath may be used as addition agents or "catalysts" in place of the sulfonic acids themselves. Unless otherwise expressly indicated, therefore, the expression "sulfonic acid" is to be understood broadly to include both the free acids and salts thereof.

The amount of organic addition agent or cata-

lyst which is desirably employed in practicing the invention may vary, in the case of the free sulfonic acids, for example, from 1 gram per liter up to saturation. Generally speaking, lowering the pH of the bath increases the solubility of the addition agents.

Deposits of even greater brightness are obtainable when the plating solution contains not only an organic addition agent but also a small quantity of either cadmium or zinc; and such conjoint use of such materials in plating solutions, particularly in nickel plating, is an important feature of the present invention. The addition to a dull nickel plating solution of a small amount of a soluble compound of an assistant or promoter metal, e. g. cadmium or zinc, for the purpose of getting some brightening effect, was long ago proposed but did not result in production of satisfactory plating deposits. As is well known, that use as heretofore proposed was too ineffective and too unsafe to be practical, especially under the operating conditions characterizing modern high-speed plating practice; and no way of overcoming the difficulties was known. But by employing a promoter metal in a nickel plating bath in conjunction with an organic brightening agent in accordance with the principles of the present invention, nickel plate of any desired thickness and of exceptional brightness may be easily produced, such deposits also being highly satisfactory in respect to their other required properties, including adequate ductility and good adherence. The promoter metal, which may be defined for the purposes of this invention as a metal having the effect, when used by itself in a bath from which a nickel group metal is electrodeposited, of enhancing the brightness of the plating metal deposited but tending to render it brittle and non-adherent, is usually added in the form of the sulfate although the specific method of adding it is in general immaterial. For example, the metal chloride may be employed, the oxide may be dissolved in the acid bath, or the metal to be introduced into the solution by dissolving it from an anode. It may also be used in the form of its compound with the sulfonic acid (e. g.) used as the principal addition agent or "catalyst". For example, excellent results are obtainable from a plating solution containing one of the organic addition agents or catalysts before mentioned together with from a trace up to about 1.6 grams of zinc per liter of solution, expressed as metal. Likewise, excellent results are obtained by the use of cadmium as the promoter in concentrations ranging from a trace upward to about 2.3 grams per liter, expressed as metal. Because these promoters, even when employed in accordance with the present invention, have the property of reducing the ductility of the resultant electrodeposits somewhat as their concentration is increased, the concentration of either of them in a given solution should be adjusted in accordance with the degree of ductility required in the electrodeposited metal.

In order to further illustrate the principles of the invention, a few detailed examples illustrating typically good practice in employing the invention will now be given. In these examples, the plating metal to be deposited is nickel, and the composition of the bath, save for the addition of assisting agents in accordance with the present invention, may be as in the ordinary and well known practice. One such typical bath composition may be approximately 320 grams

nickel sulphate and 12 grams nickel chloride per liter, with boric acid present as a buffering agent in concentration equal to about 31 grams per liter. A bath of this general constitution is particularly suitable because it is a type of nickel plating solution in widespread use on account of its desirable characteristics when operated to produce relatively thick deposits rapidly. In the examples given hereinafter, it will be assumed that a bath of this general composition is employed. Another typical bath composition which may be successfully employed, however, comprises 293 grams nickel sulphate, 12 grams nickel chloride and 25.5 grams nickel acetate, per liter, the last mentioned compound being relied upon for buffering effect. When operated in accordance with the examples hereinafter given, bright and relatively thick nickel plates or deposits of excellent character are obtained from such baths.

#### Example 1

Employing 2 amino toluene 5 sulfonic acid as the organic addition agent at a concentration of about 24 grams per liter of the plating solution (a range of about 9 to 24 grams per liter is practical), the best pH range for bright deposits of satisfactory character is approximately from 2.2 to 4.25, operating at about 50 amperes per square foot cathode current density and a bath temperature of about 40° C. For best results, the practical desirable range of cathode current density for bright deposits at pH 2.4 and bath temperature of 40° C. can be taken as approximately from 30 to 75 amperes per square foot.

#### Example 2

Using 2 amino toluene 4 sulfonic acid as the addition agent, in place of the 2-5 acid employed in Example 1, but with the plating solution otherwise similarly constituted, a range of from 10 to 20 grams of the addition agent per liter works well, about 12 grams being optimum. At this optimum concentration, the best working conditions are as follows (approximately): pH 2.0 to 5.0, cathode current density 20 to 50 amperes per square foot, and temperature 40° to 50° C.

#### Example 3

Again employing the general type of plating bath of Example 1, but using 4 amino toluene 2 sulfonic acid as the addition agent at an optimum concentration of 4 grams per liter (a range of 4 to 12 grams per liter being practical), the best pH working range for bright deposits, with a cathode current density of 50 amperes per square foot and bath temperature of 40° C., is approximately 2.5 to 5.2. At pH 2.5 and bath temperature 40° C., the most desirable practical range for bright deposits may be taken as approximately from 30 to 75 amperes per square foot.

#### Example 4

In this case, ortho-tolidine disulfonic acid is used as the organic addition agent or catalyst at a concentration lying most desirably between about 6 and 12 grams per liter. Within this concentration range, bright deposits of satisfactory character are obtained when operating at pH 2.0 to 3.0, cathode current density 40 to 60 amperes per square foot, and bath temperature 40° to 50° C.

#### Example 5

By including in the baths employed in each of the foregoing examples a promoter metal in

the form of a soluble salt thereof, in addition to the organic addition agent, the resultant plates or deposits are noticeably brighter and also satisfactory in other respects. When employing cadmium as the promoter metal, particularly good results are obtained at a concentration in the neighborhood of 0.2 gram per liter expressed in terms of the metal. When zinc is employed as the promoter, concentrations up to 10 about 1 gram per liter are found to be very satisfactory. Increase of the zinc concentration to as high as 3 grams per liter tends to cause brittleness in the deposit, and any addition of zinc as a promoter should therefore desirably be kept 15 safely below this concentration for best results. This tendency to cause brittleness is less marked in the case of zinc, however, than in the case of cadmium. The promoter metal may be conveniently added in the form of a soluble salt, 20 such as the sulfate or chloride. In general, with lower concentrations of the plating metal in the bath, the concentration of the promoter metal should also be lower, although not necessarily proportionately lower. In general, the concentration 25 of the promoter metal dissolved in the bath should not substantially exceed one-tenth normal

$$\left(\frac{N}{10}\right)$$

30 In the foregoing examples, the concentration of the plating metal in the bath is specified as approximately 2.5 N in each instance as illustrative of typical good practice, and the amounts of 35 the various addition agents or "catalysts" specified are generally indicative of satisfactory concentrations thereof in such plating baths. It is to be understood, however, that considerable variation from these optimum concentrations 40 and other operating conditions is permissible within the scope of the invention in its broader aspects.

It is found that during the plating operation 45 the addition agents or "catalysts" and/or promoters may in some cases become concentrated at the surfaces of the cathodes or work being plated. When the work is removed from the bath and rinsed, therefore, such addition agents are removed from the solution at a more rapid 50 rate, relatively, than are the other constituents of the plating bath. Accordingly, in order to compensate for the drag-out in the maintenance 55 of the bath in such cases, it is necessary to add relatively larger proportions of the "catalyst" and promoter in respect to the other materials, than are used in making up a new solution or bath. The correct proportions may be found by 60 chemical analysis or other suitable tests, and will vary with the amount of solution drag-out per ampere hour of plating.

The plating baths containing the addition agents or "catalysts" herein referred to have better throwing power than the same solutions not containing them; that is, such baths produce 65 upon an irregularly shaped article a plate of more nearly uniform thickness than do baths not containing them.

The use of the organic compounds hereinabove specifically named, as addition agents in 70 plating baths, is believed to be broadly novel irrespective of the quantity or concentration thereof in such baths or of the other plating conditions under which such baths are employed.

The deposits obtained when using a promoter 75 metal in conjunction with a sulfonic addition

agent or "catalyst" as in Example 5 hereinabove, are found upon analysis to contain in the neighborhood of 0.08 per cent carbon and 0.04 per cent sulphur, together with a larger percentage of the promoter metal. In typical instances, 5 where zinc is used as the promoter, the percentage thereof in the deposit may be about 4.3, and where cadmium is the promoter, the percentage thereof may be around 0.8.

This application is a division of my prior co- 10 pending application Serial No. 740,021, filed August 15, 1934.

What is claimed is:

1. The process of producing bright or mirror-like deposits of nickel which comprises electro-depositing nickel from an aqueous acid bath containing it mainly in the form of an inorganic salt, with the aid of a brightener comprising a toluidine sulfonic acid in quantity too small to bind chemically more than a small proportion of 20 the nickel present in the bath.

2. The process of producing bright or mirror-like deposits of nickel which comprises electro-depositing nickel from an aqueous acid bath containing it mainly in the form of an inorganic salt, with the aid of a brightener comprising an ortho toluidine sulfonic acid in quantity too small to bind chemically more than a small proportion of the nickel present in the bath.

3. The process of producing bright or mirror-like deposits of nickel which comprises electro-depositing nickel from an aqueous acid bath containing it mainly in the form of an inorganic salt, with the aid of a brightener comprising a toluidine sulfonic acid in quantity too small to bind chemically more than a small proportion of the nickel present in the bath.

4. The process of producing bright or mirror-like deposits of nickel which comprises electro-depositing nickel from an aqueous acid bath containing it mainly in the form of an inorganic salt, with the aid of a brightener comprising an ortho toluidine sulfonic acid in quantity too small to bind chemically more than a small proportion of the nickel present in the bath.

5. The process of producing bright or mirror-like deposits of a nickel group metal which comprises electrodepositing such metal from an aqueous acid bath containing the same mainly in the form of an inorganic salt, with the aid of a brightener selected from the group consisting of the following: 2 amino toluene 4 sulfonic acid, 2 amino toluene 5 sulfonic acid, 4 amino toluene 2 sulfonic acid, o-toluidine disulfonic acid, products resulting from mild chlorination thereof, and salts of the foregoing, the quantity of such brightener employed being too small to bind chemically more than a small proportion of the nickel group metal present in the bath.

6. The process of producing bright or mirror-like deposits of nickel which comprises electro-depositing nickel from an aqueous acid bath containing the same mainly in the form of an inorganic salt, with the aid of a brightener selected from the group consisting of the following: 2 amino toluene 4 sulfonic acid, 2 amino toluene 5 sulfonic acid, 4 amino toluene 2 sulfonic acid, o-toluidine disulfonic acid, products resulting from mild chlorination thereof, and salts of the foregoing, the quantity of such brightener employed being too small to bind chemically more than a small proportion of the nickel present in the bath.

7. The process of producing bright or mirror-like deposits of nickel of substantial thickness (i. e. more than 0.0002 inch) and characterized by 75

good adherence and substantial freedom from cracking or curling, which comprises electrodepositing nickel from an aqueous acid bath containing the same mainly in the form of an inorganic salt, with the aid of a brightener comprising a water-soluble sulfonated amino toluene compound employed in quantity too small to bind chemically more than a small proportion of the nickel present in the bath, and a promoter metal, employed at a concentration not substantially exceeding one-tenth normal

$$\left(\frac{N}{10}\right)$$

cooperating with said brightener to enhance the brightening effect.

8. The process defined in claim 1, further characterized by the fact that said bath contains a promoter metal, employed at a concentration not substantially exceeding one-tenth normal

$$\left(\frac{N}{10}\right)$$

cooperating with said brightener to enhance the brightening effect.

9. The process defined in claim 3, further characterized by the fact that said bath contains a promoter metal, employed at a concentration not substantially exceeding one-tenth normal

$$\left(\frac{N}{10}\right)$$

cooperating with said brightener to enhance the brightening effect.

10. The process of producing bright or mirror-like nickel plating of substantial thickness (i. e. more than 0.0002 inch) and characterized by good adherence and substantial freedom from cracking or curling, which comprises electrodepositing nickel from an acidic aqueous plating bath containing it in the form of an inorganic salt, together with a brightener selected from the group consisting of the following: 2 amino toluene 4 sulfonic acid, 2 amino toluene 5 sulfonic acid, 4 amino toluene 2 sulfonic acid, o-tolidine disulfonic acid, products resulting from mild chlorination thereof, and salts of the foregoing, the quantity of such brightener employed being too small to bind chemically more than a small proportion of the nickel group metal present in the bath; and a promoter metal cooperating therewith to enhance the brightening effect and employed at a concentration not substantially exceeding one-tenth normal

$$\left(\frac{N}{10}\right)$$

11. The process defined in claim 10, further characterized by the fact that the promoter metal is selected from the group consisting of cadmium and zinc.

12. The process defined in claim 5, wherein the plating bath is maintained at a temperature between 35° and 60° C., most desirably between 40° and 50° C., and at a pH between 5.5 and 1.5, most desirably at about 2.5, and is operated at a cathode current density of between 10 and 100 amperes, most desirably between 30 and 50 amperes, per square foot.

13. The process defined in claim 6, wherein the plating bath is maintained at a temperature between 35° and 60° C., most desirably between 40° and 50° C., and at a pH between 5.5 and 1.5, most desirably at about 2.5, and is operated at a cathode current density of between 10 and 100 amperes, most desirably between 30 and 50 amperes, per square foot.

14. An electroplating bath for producing a bright deposit of a nickel group metal which comprises an acidic aqueous solution of a compound of a nickel group metal, together with a brightener selected from the group consisting of the following: 2 amino toluene 4 sulfonic acid, 2 amino toluene 5 sulfonic acid, 4 amino toluene 2 sulfonic acid, o-tolidine disulfonic acid, products resulting from mild chlorination thereof, and salts of the foregoing, the quantity of such brightener employed being too small to bind chemically more than a small proportion of the nickel group metal present in the bath.

15. An electroplating bath for producing a bright deposit of a nickel group metal of substantial thickness (i. e. more than 0.0002 inch) and characterized by good adherence and substantial freedom from cracking or curling, which comprises an acidic aqueous solution of a compound of a nickel group metal, together with a water soluble sulfonated amino toluene compound brightening agent, and a small quantity of a promoter metal added to the bath to enhance the brightness of the electrodeposit obtainable therefrom, the concentration of said promoter metal not substantially exceeding one-tenth normal

$$\left(\frac{N}{10}\right)$$

16. An electroplating bath for producing bright nickel plating of substantial thickness (i. e. more than 0.0002 inch) and characterized by good adherence and substantial freedom from cracking or curling, which comprises an aqueous solution containing nickel mainly in the form of an inorganic salt, together with a sulfonated amino toluene compound brightening agent in quantity too small to bind chemically more than a small proportion of the nickel present in the bath, and a promoter metal adapted to cooperate with said sulfonated compound to enhance the brightening effect and employed at a concentration not substantially exceeding one-tenth normal

$$\left(\frac{N}{10}\right)$$

said bath having a pH value of between 1.5 and 5.5.

17. An electroplating bath for producing bright nickel plating of substantial thickness (i. e. more than 0.0002 inch) and characterized by good adherence and substantial freedom from cracking or curling, which comprises an aqueous solution having an acid reaction and containing nickel mainly in the form of an inorganic salt, together with an organic brightener selected from the group consisting of the following: 2 amino toluene 4 sulfonic acid, 2 amino toluene 5 sulfonic acid, 4 amino toluene 2 sulfonic acid, o-tolidine disulfonic acid, products resulting from mild chlorination thereof, and salts of the foregoing, the quantity of such brightener employed being too small to bind chemically more than a small proportion of the nickel group metal present in the bath; together with a promoter metal adapted to cooperate with said sulfonated compound to enhance the brightening effect and employed at a concentration not substantially exceeding one-tenth normal

$$\left(\frac{N}{10}\right)$$

18. An electroplating bath as defined in claim 17, wherein the promoter metal is selected from the group consisting of cadmium and zinc.